

UNITED STATES PATENT OFFICE

2,627,512

## COPOLYMERS OF ACRYLONITRILE WITH N-ACROYL N'-ALANYL METHYLENE DIAMIDES

Ernst Zerner and Mark W. Pollock, New York, N. Y., assignors to Sun Chemical Corporation, Long Island City, N. Y., a corporation of Delaware

**No Drawing. Application July 20, 1951,  
Serial No. 237,822**

5 Claims. (CL 260—85.5)

三

The present invention relates to copolymers of acrylonitrile which are adapted to be formed into fibers, films and the like and which are further particularly retentive of conventional dyestuffs.

It is well known that polyacrylonitrile has properties which make this material commercially valuable. For example, polyacrylonitrile may be cast into self-supporting films or may be spun from solutions thereof to provide fibers which are capable of being cold drawn, whereby the structure of the fiber is molecularly oriented along the axis of the fiber to produce fibrous materials of high tensile strength. These materials are further insensitive to water and to the common organic solvents usually employed in dry cleaning operations. Therefore, such fibrous materials have been found to be suitable for use in many of the applications in which the common textile fibers are employed, and have further been found to provide more durable end products.

However, despite the seemingly apparent advantages of polyacrylonitrile fibers over those generally employed in the textile field, the use of the same in textile applications has been limited due to the insensitivity of these materials to the conventional dyes employed to color fibers and fabrics of the ordinary textile materials such as cotton, rayon, etc. If, however, it were possible to provide polyacrylonitrile fibers, or fibers having all of the desirable and advantageous properties of polyacrylonitrile fibers, which fibers also displayed an affinity for conventional dyes and which were further retentive of such dyes, then it is believed that such fibers would in all probability find wide commercial use in the field of textiles and would prove to be extremely valuable in many such applications.

The art discloses that various copolymers of acrylonitrile have been prepared to meet this purpose. For example, U. S. P. No. 2,491,471 discloses the preparation of copolymers of acrylonitrile with vinylpyridine which copolymers are said to be capable of furnishing oriented filaments of high tensile strength and also to be susceptible of being dyed with acid dyes. In U. S. P. No. 2,581,408, there are disclosed copolymerization products of acrylonitrile and itaconic acid, which products are said to be adapted to dyeing, particularly with basic dyes, and which are also adapted to the formation of molecularly oriented shaped articles. In each of these cases, however, the copolymer obtained with the materials set forth therein is comparatively expensive. Therefore, one object of the present invention is to provide acrylonitrile copolymers which may be readily

cast into self-supporting films or formed into molecularly oriented fibers, which are adapted to be dyed with conventional dyes and which are highly retentive of such dyes, and which further-  
5 more are relatively inexpensive to produce.

The above object is accomplished, according to the present invention, by copolymerizing acrylonitrile with N-acryloyl N'-alanyl methylene diamides, corresponding to the general formula

10



15 where R is a member of the group consisting of hydrogen and methyl, and where Y is the residue of a compound selected from the group consisting of aliphatic amines, alicyclic amines and heterocyclic amines, which amines have at least one hydrogen attached to the amino nitrogen thereof,  
20 the point of attachment of the said residue being at the amino nitrogen thereof. The copolymers thus formed are particularly receptive of acidic dyes.

Methylene diamides of the above type are described in a copending application Serial No. 25 85,038, filed April 1, 1949, in the name of Philip P. Dalton, and now abandoned. As described therein, such compounds may be prepared by reacting a methylene-bis-acrylamide corresponding to the formula:

60



where R represents hydrogen or a methyl radical, with a primary or secondary aliphatic amine under such conditions that saturation of only one of the terminal unsaturated groups of the methylene-bis-acrylamide by the amine is effected. The compounds thus formed may be considered to be 40 amine mono-addition products of the methylene-bis-acrylamides. By selectively effecting the reaction between the amines and the methylene-bis-acrylamides such that saturation of only one of the terminal unsaturated groups of the methylene-bis-acrylamides is effected, the resulting addition products are capable of undergoing further reaction involving copolymerization of the addition products with other polymerizable monomers.

50 In accordance with the present invention we have found that those methylene-bis-acrylamides in which only one of the terminal unsaturated groups thereof has been converted into a saturated grouping by reaction with aliphatic, alicyclic or heterocyclic amines, which amines have at

least one hydrogen atom attached to the amino nitrogen atom thereof, may be reacted with acrylonitrile to furnish copolymerization products which may readily be formed into molecularly oriented fibers and which are readily receptive and retentive of conventional acid dyes. The copolymerization products of the present invention contain principally acrylonitrile, the ratio of acrylonitrile to the amine mono-addition products of the methylene-bis-acrylamides employed being generally within the range of approximately 90% to 99% by weight of acrylonitrile to approximately 10% to 1% by weight of the said amine mono-addition products.

Illustrative of various amines which may be utilized to provide the amine mono-addition products of the methylene-bis-acrylamides employed in preparing the copolymers of the present invention are methylamine, ethylamine, butylamine, decylamine, benzylamine, phenylethylamine, monoethanolamine, diethylamine, diethanolamine, cyclohexylamine, morpholine, piperidine and pyrrolidine. The term "aliphatic amine" as utilized in the present invention refers to amines in which the amino group is attached to an aliphatic group.

Preparation of the amine mono-addition products of the methylene-bis-acrylamides and the subsequent copolymerization thereof with acrylonitrile are illustratively set forth in the following examples. All proportions are given in parts by weight.

*Example 1.—Formation of the diethylamine mono-addition product of methylene-bis-acrylamide*

In a suitable reaction vessel there are placed 4.6 parts of methylene-bis-acrylamide dissolved in a mixture of 70 parts water and 40 parts acetone. To this solution there is slowly added with stirring a solution of 2.2 parts of diethylamine in a mixture of 2 parts acetone and 8 parts water. The complete mixture is then heated at a temperature of 40° to 50° C. for approximately 3 hours to insure substantially complete reaction between the reacting materials. The reaction mixture is then allowed to stand for approximately 24 hours, after which time it is filtered to remove any insoluble material which may be present. The filtrate is then allowed to evaporate to dryness, there being obtained approximately 6.8 parts of a material consisting essentially of a compound corresponding to the formula



In the above example, as in each of the illustrative examples describing the formation of the addition products of the methylene-bis-acrylamides, a 20% excess of the amine above the theoretical molecular amount required to effect the desired reaction is employed to avoid the possible presence in the reaction product of unreacted methylene-bis-acrylamide.

*Example 2*

One part of the product obtained in Example 1 was dissolved in 19 parts of freshly distilled acrylonitrile and the solution was then added to a solution of 0.4 part of ammonium persulfate and of 0.1 part of sodium bisulfite in 180 parts water. The pH of this solution was then adjusted to a pH value of 3 to 4 with dilute sulfuric acid. The solution thus obtained was heated

for approximately 3 hours at a temperature of 50°-60° C. and was then allowed to cool and to stand at room temperature with occasional agitation for two days. At the end of this time a white precipitate had formed which was separated by filtration and air-dried. The material thus obtained was a copolymer containing approximately 95% by weight of acrylonitrile and approximately 5% by weight of the diethylamine mono-addition product of methylene-bis-acrylamide.

A self-supporting film of the copolymer of Example 2, obtained by casting the same from a solution of the copolymer in dimethyl formamide, was immersed for approximately one-half hour in a boiling aqueous solution of Alizarine Saphire SE, an acid dye manufactured by the National Aniline Division of Allied Chemical and Dye Corporation. At the end of this time, the copolymer film was found to be dyed a deep blue color. A film of polyacrylonitrile, treated in the same manner, was completely unaffected by the dye.

*Example 3*

Formation of the butylamine mono-addition product of methylene-bis-methacrylamide.

Following the procedure set forth in Example 1 except that a reaction mixture is employed which consists of a solution of 18.2 parts of methylene-bis-methacrylamide in a mixture of 280 parts of water and 160 parts of acetone and to which solution a solution of 8.8 parts of butylamine in a mixture of 8 parts of acetone and 32 parts of water has been added, there is secured a product which consists essentially of a compound corresponding to the formula



*Example 4*

A copolymer of acrylonitrile and the butylamine mono-addition product of methylene-bis-methacrylamide was prepared in accordance with the procedure set forth in Example 2 utilizing 0.5 part of the product of Example 3 to 19.5 parts of acrylonitrile. The copolymer thus obtained was one containing approximately 2.5% by weight of the butylamine mono-addition product of methylene-bis-methacrylamide to 97.5% by weight of acrylonitrile.

A film, cast from a solution of such copolymer in dimethyl formamide and subjected to treatment for approximately one-half hour in a boiling aqueous solution of the acid dye mentioned hereinbefore, acquired a permanent blue color.

*Example 5.—Formation of the morpholine mono-addition product of methylene-bis-acrylamide*

To a solution of 15.4 parts of methylene-bis-acrylamide dissolved in a mixture of 280 parts of water and 160 parts of acetone there are added 10.5 parts of morpholine dissolved in 40 parts of a 20% acetone in water solution. The reaction is then carried out in accordance with the procedure set forth in Example 1, the product thus secured consisting essentially of a material corresponding to the formula



## Example 6

Following the procedure set forth in Example 2, one part of the product of Example 5 is reacted with 19 parts of acrylonitrile to provide a copolymer containing approximately 95% by weight of acrylonitrile and approximately 5% by weight of the morpholine mono-addition product of methylene-bis-acrylamide. The copolymer thus obtained exhibited the same dye-receptive properties characteristic of the copolymers of the present invention.

## Example 7.—Formation of the cyclohexylamine mono-addition product of methylene-bis-acrylamide

The procedure set forth in Example 1 is followed except that, as the reaction mixture, there is employed a solution of 15.4 parts of methylene-bis-acrylamide in a mixture of 280 parts of water and 160 parts of acetone to which solution there was added a solution of 11.9 parts of cyclohexylamine in 40 parts of a 50% acetone-water mixture. The product resulting from such reaction is a material which consists essentially of a compound corresponding to the formula



## Example 8

A copolymer containing approximately 95% by weight of acrylonitrile and approximately 5% by weight of the cyclohexylamine mono-addition product of methylene-bis-acrylamide is obtained by reacting one part of the product of Example 7 with 19 parts of acrylonitrile in accordance with the process set forth in Example 2. The copolymer thus formed is characterized by its affinity for acid dyes.

As has been stated hereinbefore, the copolymerization products of the present invention contain principally acrylonitrile. The amount, with respect to the acrylonitrile, in which the amine mono-addition products of the methylene-bis-acrylamides should be utilized in preparing the copolymers will depend upon the qualities desired in the finished product. It has been found that an amount of the mono-addition product corresponding to at least 1% by weight of the acrylonitrile should be used to provide copolymers which are particularly receptive of acid dyes. The receptivity or affinity of the copolymers of the present invention for such dyes appears to increase as the ratio of the mono-addition products to acrylonitrile in the copolymers increases. However, for best results, it is not preferred to employ amounts of the mono-addition product substantially in excess of 10% by weight of the acrylonitrile since there is no particular advantage to be gained in the use of such amounts of the mono-addition product, and due to the further fact that such amounts of the mono-addition product tend to change the character of the copolymer obtained.

The copolymers of the present invention may be cast into strong, flexible, self-supporting films or may be spun into fibers which may be molecularly oriented as by cold drawing to provide fibers of high tensile strength. The solvents ordinarily employed in dry cleaning operations have no appreciable effect upon either the copolymers themselves or upon the color imparted to these

materials when they are dyed in accordance with the methods hereinbefore set forth. Therefore, fibers prepared from the copolymers of the present invention are of obvious utility in the manufacture of wearing apparel, and have particular utility as a partial replacement for wool.

While the above products and processes of preparing the same constitute preferred embodiments of the present invention, changes may be made therein without departing from the scope of the invention as defined in the appended claims.

## What is claimed is:

1. As a new product, a copolymerization product of from 90% to 99% by weight of acrylonitrile with from 10% to 1% by weight of a compound of the general formula



where R is a member of the group consisting of hydrogen and methyl, and where Y is the residue of a compound selected from the group consisting of aliphatic amines, alicyclic amines, and heterocyclic amines, the said amines having at least one hydrogen attached to the amino nitrogen atom, the point of attachment of the said residue being at the amino nitrogen thereof.

2. As a new product, a copolymerization product of from 90% to 99% by weight of acrylonitrile with from 10% to 1% by weight of a compound of the formula



3. As a new product, a copolymerization product of from 90% to 99% by weight of acrylonitrile with from 10% to 1% by weight of a compound of the formula



4. As a new product, a copolymerization product of from 90% to 99% by weight of acrylonitrile with from 10% to 1% by weight of a compound of the formula



5. As a new product, a copolymerization product of from 90% to 99% by weight of acrylonitrile with from 10% to 1% by weight of a compound of the formula



ERNST ZERNER.  
MARK W. POLLOCK.

## REFERENCES CITED

The following references are of record in the file of this patent:

## UNITED STATES PATENTS

| Number    | Name   | Date          |
|-----------|--------|---------------|
| 2,478,378 | Dickey | Aug. 9, 1949  |
| 2,576,501 | Dalton | Nov. 27, 1951 |